

## UNITED STATES PATENT OFFICE

2,607,734

## PROCESS OF MANUFACTURING HYDROXY ACID GREASES AND PRODUCT THEREOF

Lorne W. Sproule, Sarnia, Warren C. Pattenden, Courtright, and Laurence F. King, Sarnia, Ontario, Canada, assignors to Standard Oil Development Company, a corporation of Delaware

No Drawing. Application May 20, 1950,  
Serial No. 163,328

6 Claims. (Cl. 252—39)

1

The present invention relates to an improved process of preparing lubricating greases and, particularly, greases containing soaps of hydroxy acids, such as 12-hydroxy stearic acid. In particular, it relates to a process by which stable calcium base greases of superior consistency may be prepared under conditions of dehydration as contrasted to the conventional hydration.

In application Serial No. 81,206, filed March 12, 1949, by the present applicants, there is described a process for making stable calcium base greases suitable for high temperature use by using mono- or dihydroxy saturated fatty acids, instead of normal fatty acids, for preparing the soaps which thicken lubricating oils to grease consistency. The advantages of the hydroxy acids in the case of calcium base greases are pointed out in said application. Briefly, these greases are stable at temperatures which would evaporate the water required as a stabilizer in the older type calcium base greases. According to the present invention, superior greases of lower soap content may be obtained by improvements in processing.

The specific phenomena by which stable calcium base greases may thus be prepared under conditions of relative dehydration are not clear, but it appears that when a hydroxy fatty acid is used, which has one or two hydroxy groups attached to the chain, these hydroxy groups in some manner perform the function for which water ordinarily has been required in the standard calcium greases of the prior art. As those familiar with the art understand, conventional calcium greases must be plasticized or hydrated with a small amount of water, e. g., 0.5 to 2% by weight, based on the total grease. When operating conditions are such that this water is substantially evaporated, the conventional calcium base greases quickly lose their grease structure and become unsuitable for use.

According to the present invention, it is found that the standard method of preparing lime soap greases is not satisfactory for preparing the

greases containing calcium soaps of hydroxy acids. The normal procedure is carried out in three steps. First, the fats or fatty acids are saponified with lime, usually in the presence of 5 at least small quantities of mineral lubricating oil at a suitable temperature, for example, about 325° F. Next, the soap-oil concentrate is cooled to a temperature close to the boiling point of water, for example, about 225° F., while additional mineral oil and small quantities of water are added and stirred into the mixture. Finally, 10 additional lubricating oil is added to the soap-water-oil mixture until a grease is obtained having the desired consistency. This product is then cooled to a suitable drawing temperature, for example, about 175° F., and is drawn into receptacles or packages.

During the first or saponification stage, the 15 soap is in a semi-fluid state. If it is allowed to cool to 175° F. or so without addition of further oil or water it forms a dry, hard, brittle mass. When water is incorporated as in the second step given above, the soap-oil mixture forms a soft plastic composition of grease-like structure. If 20 the product of the first step is merely diluted with oil and cooled, for example, to about 175° F. or so without the addition of water, the soap and oil will separate into two phases. This heterogeneous product is quite worthless as a grease, and its components cannot be dispersed in each other to form a real grease even by drastic mechanical working.

According to the present invention, although 25 the greases containing hydroxy acids can be made substantially anhydrous, care must be taken in dehydrating them. If the soap stock or concentrate is merely heated in a small amount of oil to a temperature of about 300° F. or so 30 and the product is then allowed to cool, the soap will separate almost entirely from the lubricating oil. This separation occurs at a temperature of about 275° F. and the soap cannot be subsequently dispersed in the oil, even by the 35 addition of water followed by agitation.

For purposes of the present invention, a preferred process by which a superior grease can be prepared is as follows: The hydroxy fatty acid, which may be 12-hydroxy stearic acid or other mono- or dihydroxy fatty acids having from about 12 to 24 carbon atoms, is reacted with lime at a temperature of about 180° to 200° F., preferably about 190° F. The hydroxy acid and lime are preferably reacted in the presence of a relatively small amount of oil, for example, about 1/2 to 5 times as much oil, by weight, as hydroxy acid. The oil used is ordinarily mineral base lubricating oil of appropriate viscosity for the service for which the grease is prepared, i. e., between 60 and 5,000, preferably about 100 to 1,000 S. U. S. at 100° F. The quantity of lubricating oil preferably should be from about equal to about four times the weight of the hydroxy acid. After the hydroxy acid and lime have thus been reacted in the presence of lubricating oil, the mass is slowly heated for slow and controlled dehydration, with continuous stirring, to a maximum temperature of about 250° to 300° F., preferably not above about 275° F. The maximum temperature specifically preferred, especially for 12-hydroxy stearic acid, which is a preferred acid although others can be used, is about 265° to 270° F. At such temperatures, the mixture is gradually dehydrated and after the water is removed, further lubricating oil is gradually added with continued stirring. As the temperature begins to drop, a grease of suitable structure readily forms. The remainder of the lubricating oil is then added while the grease is further cooled, with continued stirring, to a temperature of about 180° to 210° F., preferably below 200° F. At the latter temperature, the grease may be drawn into packages or other containers. The finished product is not necessarily absolutely dry or anhydrous, but is substantially so. It may contain up to about 0.1% by weight of water, though a smaller water content, not greater than 0.05%, is preferred. Water is not an essential ingredient and ordinarily none is added intentionally, as it must be in the prior art processes of preparing conventional calcium base greases.

The invention will be described further with reference to specific examples.

#### EXAMPLE I

150 lbs. of 12-hydroxy stearic acid (commercial grade) were charged to a 4000 lb. steam-jacketed kettle and 570 lbs. of mineral oil (V./100° F.: 300 S. U. S.; V. I.: 54) added. The mixture was stirred and heated to 190° F. to obtain solution of the fatty acid in the oil.

22 lbs. of hydrated lime in the form of a slurry with about 80 lbs. of water were added to the fatty acid-oil solution and the mixture stirred for 1/2 hour. The contents were then allowed to stand for 10-18 hours, although it is not believed that this standing time is essential to the process.

Stirring was commenced and steam was applied to the kettle jacket through a pressure regulator. It was found necessary to control the steam pressure at 20-25 p. s. i. g. in order to avoid overheating or too rapid dehydration of the soap at the kettle walls.

Dehydration was carried out, the maximum temperature being about 250° F. This process required about 14 hours. The following table

shows the increase in consistency which accompanied dehydration.

| Percent Water in Grease (by distillation with Xylene) | Worked Penetration (77° F.) |
|-------------------------------------------------------|-----------------------------|
| 0.5                                                   | 330                         |
| 0.45                                                  | 308                         |
| 0.4                                                   | 280                         |
| 0.3                                                   | 250                         |
| 10 0.3                                                | 236                         |
| 0.2                                                   | 197                         |
| 0.1                                                   | 160                         |
| 0.05                                                  | 142                         |

When dehydration was finished, further oil (1400 lbs.) was worked into the soap stock until the worked penetration was 285/77° F. At this stage, the grease contained about 7% of 12-hydroxy stearic acid in the form of the calcium soap.

From Example I, the following points will be noted:

(1) The process is essentially one of dehydration accompanied by mechanical shearing or milling. This is directly opposite to the manufacture of conventional lime soap grease which require hydration with 0.5 to 2% of water in order to obtain a stable dispersion of the soap.

(2) If the soap stock is not completely or substantially completely dehydrated, a grease of low yield is obtained. The water content should be down to 0.05% or less. Otherwise, an important advantage of the present invention, the reduction in soap requirements to attain a given consistency, is largely lost. In order to illustrate this, a portion of the soap stock (concentrate) of Example I, showing a worked penetration of 197 mm./10 with a water content of 0.2% was diluted with oil to form a grease. With calculated hydroxy stearic acid content of 10.5%, a worked penetration of 308 mm./10 was obtained. This is soft for such a soap content. Furthermore, on subsequent reheating such greases tend to harden and form crusts on the surface. The discovery of the effect of very low water content led to the substantial improvement of consistency.

(3) The addition of water to a calcium hydroxy stearate grease, after manufacture is completed, does not affect the consistency of the grease appreciably. Hence, inadvertent addition of moisture at a later stage is not particularly objectionable.

(4) On the other hand, if a sample of soap stock, such as the concentrate of Example I, containing 0.2% water as above, is dehydrated in an oven at 250° F. without stirring, a product containing many hard lumps of soap is obtained. This illustrates the necessity of agitation during the dehydration.

#### EXAMPLE II

Another grease was prepared by the same method as the grease of Example I, except that an oil of higher viscosity was used. The ingredients are indicated in Table I where comparative tests with and without milling are shown of both greases, Examples I and II. Results indicated that milling of the greases resulted in considerable improvement in their characteristics. The wheel bearing test showed considerable leakage in the unmilled grease of Example I. The milled grease showed no leakage whatever. Milling was found to improve the viscosity and bleeding properties as well as to improve performance in the wheel bearing test.

Table I

## PROPERTIES OF CALCIUM HYDROXY STEARATE GREASES

| Grease                                                | Example I | Example II |
|-------------------------------------------------------|-----------|------------|
| Formula, percent by weight:                           |           |            |
| 12-Hydroxy Stearic Acid.....                          | 7.0       | 6.40       |
| Hydrated Lime.....                                    | 1.0       | 0.95       |
| LCT 20 Base (V./100° F.: 300; V. I. 54) <sup>1</sup>  | 91.5      | 24.60      |
| LCT 40 Base (V./100° F.: 1350; V. I. 54) <sup>1</sup> |           | 68.05      |
| Phenyl Alpha Naphthylamine.....                       | 0.5       |            |

<sup>1</sup> Low Cold Test Mineral Oil.

| Inspections                                             | No Milling       | Through Colloid Mill | No Milling       | Through Colloid Mill |
|---------------------------------------------------------|------------------|----------------------|------------------|----------------------|
| Mineral Oil V./210° F. S. U. S.....                     | 50               | 50                   | 72               | 72                   |
| Penetration.....                                        | 286              | 290                  | 290              | 265                  |
| Worked Penetration 77° F.....                           | 284              | 286                  | 279              | 279                  |
| A. S. T. M. Dropping Point °F.....                      | 291              | 289                  | 297              | 292                  |
| Bleeding—Percent Oil Loss<br>(100 hrs. at 225° F.)..... | 9.7              | 7.0                  | 8.9              | 6.0                  |
| Apparent Viscosity at 100 sec-1 (Stokes):               |                  |                      |                  |                      |
| 77° F.....                                              | 84               | 91                   | 107              | 127                  |
| 130° F.....                                             | 33               | 43                   | 37               | 49                   |
| 175° F.....                                             | 20               | 27                   | 21               | 29                   |
| 200° F.....                                             | 14               | 20                   | 17               | 22                   |
| 225° F.....                                             | 11               | 15                   | 13               | 17                   |
| 250° F.....                                             | 8.5              | 10                   | 9                | 9                    |
| 275° F.....                                             | 4.2              | 3.8                  | 3                | 4                    |
| 300° F.....                                             | ( <sup>2</sup> ) | ( <sup>3</sup> )     | ( <sup>3</sup> ) | ( <sup>3</sup> )     |
| C. R. C. Wheel Bearing Test<br>(6 hrs. at 220° F.)..... | 24.3             | 1.5                  | nil              | nil                  |
| Grease Leakage (gms.).....                              | 0.8              | nill                 | 0.4              | —                    |

<sup>2</sup> These values represent different tests on the same sample.<sup>3</sup> Separated.

## EXAMPLE III

Another calcium base grease containing 12-hydroxy stearic acid and mineral lubricating oil of about 300 S. U. S. viscosity at 100° F. was prepared in the manner described above in a conventional grease kettle. This product showed the following characteristics and inspections:

Composition percent by weight:

|                                             |      |
|---------------------------------------------|------|
| 12 - hydroxy stearic acid (comm. grade)     | 10.5 |
| Hydrated lime.....                          | 1.5  |
| Mineral oil (V. I 54; V./100° F.: 300)..... | 88.0 |

Inspections:

|                                         |     |
|-----------------------------------------|-----|
| Worked penetration 77° F. (mm./10)..... | 273 |
| A. S. T. M. Dropping Point °F.....      | 288 |

C. R. C. Wheel Bearing Test:

|                              |           |
|------------------------------|-----------|
| Grams of grease leakage..... | 0         |
| Rating.....                  | Excellent |

Upon passage of the product of Example I through a laboratory colloid mill no change in consistency was observed.

## EXAMPLE IV

Another grease composition likewise containing calcium soap of 12-hydroxy stearic acid and an oil of similar viscosity index (about 55) but of higher viscosity, about 900 S. U. S. at 100° F., was prepared in the same manner. As finished in the grease kettle, this product showed a worked penetration, after 60 strokes in the standard ASTM grease worker equipped with  $\frac{1}{4}$  inch holes, of 281 mm./10. This product contained about 9.5% by weight, based on the total composition, of the calcium soap. It was slightly grainy in structure. After one passage through the laboratory colloid mill, the grease was hardened somewhat and its graininess somewhat reduced. It showed a worked penetration of 235 mm./10. Thereafter, additional oil was stirred into the grease until the worked penetration increased to 286 mm./10. The soap content of the finished

product was about 6.1% by weight. The comparative characteristics of the grease of Example IV, the same grease after passage through the colloid mill, and the milled grease which was cut back with additional oil, are shown in the following table:

Table II

|                                                              | Example IV      | After Colloid Milling | After Thinning   |
|--------------------------------------------------------------|-----------------|-----------------------|------------------|
| Percent soap.....                                            | 9.5             | 9.5                   | 6.1              |
| Worked Penetration 77° F. (mm./10).....                      | 281             | 235                   | 286              |
| Texture.....                                                 | Slightly grainy | Smooth                | Smooth           |
| C. R. C. Wheel Bearing Test:<br>Grams of grease leakage..... | 4.4:3.5<br>Fair | No data<br>Good       | 0.1<br>Excellent |

From the data given in the above examples, the following conclusions are drawn concerning the preparation of hydroxy acid greases.

(1) The grease must be prepared at a maximum temperature not more than about 275° F., preferably about 270° F.

(2) With oils of higher viscosity, the product should be finished by milling to improve its texture. When this is done, greases of excellent properties and extremely low soap content, in view of the consistency of the product, may be obtained.

(3) In cooking the soap, dehydration should be carried out slowly. Rapid cooking seems to destroy stability.

The greases prepared above in Examples III and IV were made in 100-pound batches. Full scale plant batches were made of Examples I and II. The data based on Examples I and II are, therefore, somewhat more firm. Furthermore, the control of dehydration was better in Examples I and II.

The usual additives and modifiers, such as oxidation inhibitors, corrosion inhibitors, extreme pressure agents, and the like, may be used in the

greases of this invention, if desired, as will be obvious to those skilled in the art. Preferred types of greases usually contain from about 5 to 12% of the hydroxy acid, preferably 12-hydroxy stearic acid, in the form of the calcium soap, but proportions may be as low as 2% or as high as 30%, based on the weight of the final composition.

What is claimed is:

1. The process of preparing a substantially anhydrous lubricating grease which comprises saponifying 2 to 30% by weight, based on the total final composition, of hydroxy acid selected from the group which consists of substantially saturated mono- and dihydroxy fatty acids which range between about 12 and about 24 carbon atoms per molecule with lime in the presence of about one-half to about five times the quantity of mineral base lubricating oil based on the weight of the hydroxy acids and at a maximum cooking temperature below about 275° F., and thereafter adding additional lubricating oil as the oil-soap mixture is cooled, with continuous stirring, until a temperature of about 200° F. is reached.

2. The process according to claim 1 wherein the grease is passed through a colloid mill after cooling to improve its performance in anti-friction bearings.

3. A lubricating grease composition consisting essentially of mineral base lubricating oil having a viscosity between 60 and 5,000 S. U. S. at 100° F. and thickened to grease consistency with about 2 to 30% by weight, based on the total composition, of substantially anhydrous

calcium soap of a substantially saturated hydroxy acid selected from the group which consists of mono- and dihydroxy fatty acids having not less than 12 nor more than 24 carbon atoms per molecule, said grease being cooked to a maximum temperature not above 275° F. during soap formation.

4. The product according to claim 3 wherein the hydroxy acid is 12-hydroxy stearic acid.

5. The process of preparing a substantially anhydrous lubricating grease which comprises saponifying about 2 to 30% by weight, based on the total composition, of 12-hydroxy stearic acid, with lime at a maximum cooking temperature of 275° F., in the presence of  $\frac{1}{2}$  to 5 times as much mineral lubricating oil as acid, cooking slowly to gradually dehydrate and form a soap concentrate, and then adding further mineral oil and stirring while cooling to about 190° F.

6. Process according to claim 5 wherein the proportions of acid are between 5 and 12% by weight.

LORNE W. SPROULE.  
WARREN C. PATTENDEN.  
LAURENCE F. KING.

#### REFERENCES CITED

The following references are of record in the file of this patent:

#### UNITED STATES PATENTS

| Number    | Name            | Date           |
|-----------|-----------------|----------------|
| 2,380,960 | Fraser          | Aug. 7, 1945   |
| 2,450,224 | Bergmann et al. | Sept. 28, 1948 |
| 2,503,749 | Langer et al.   | Apr. 11, 1950  |